

## UNITED STATES PATENT OFFICE

2,306,283

## COLORATION OF TEXTILE MATERIALS

George Schneider, Montclair, N. J., assignor to  
Celanese Corporation of America, a corporation  
of Delaware

No Drawing. Application March 19, 1940,  
Serial No. 324,797

8 Claims. (Cl. 106—193)

This invention relates to the coloration of textile materials, and relates more particularly to the production of dark colors on textile materials made of or containing cellulose esters or ethers.

This invention is a continuation-in-part of the invention described in application S. No. 277,619 filed June 6, 1939.

An important object of this invention is the economic and expeditious production of an artificial material having a neutral grey color which is fast to light, acid and perspiration.

Another object of this invention is the production of an artificial textile material which is neutral grey in color and which is free from red, brown or blue fluorescence or cast.

A further object of this invention is the production with greater ease and at less expense of fast dark shades on textile materials made of or containing cellulose esters or ethers by dyeing the neutral grey colored materials, produced in accordance with this invention, by direct dyeing methods.

Other objects of this invention will appear from the following detailed description and claims.

The production of satisfactory blacks and other dark colorations on textile materials by direct dyeing methods is a matter of some difficulty. In the first place there is a decided lack of direct dyeing dyestuffs of satisfactory fastness properties, and in the second place, in order to produce shades of sufficient depth it is generally necessary to employ proportions of dyestuff relative to the material which are very high as compared with those usually sufficient for the production of pale or medium shades. As a consequence the deep dyeings produced by direct dyeing methods frequently lack fastness to rubbing in addition to lacking fastness to other agencies. Furthermore, the use of such high proportions of coloring matters involves considerable expense. Consequently, if satisfactory deep shades are required, it has generally been found expedient to employ indirect dyeing methods such as dyeing with vat dyestuffs or with azo dyestuffs produced on the material. These latter methods, however, suffer from the grave disadvantage that they require exceptional skill and that the matching of shades to a given sample is a matter of some difficulty.

The aforesaid difficulties are particularly pronounced in the case of cellulose ester or ether materials owing to the substantial absence of any direct dyeing unitary dyestuffs capable of yielding black or other dark shades thereon. If,

therefore, it is desired to produce such dark shades by direct dyeing methods, it has been essential to employ very large proportions of mixtures of brightly dyed dyestuffs. Thus, black shades have been produced by the application of a mixture of direct dye blue, red and orange or yellow dyestuffs in which the blue predominates. Such dyeings are particularly prone to lack fastness to rubbing.

It has been proposed to incorporate in textile materials a dark colored pigment of such character and in such proportion as to yield thereon a grey, drab or other dark shade and then subsequently dyeing these materials by direct dyeing methods to produce a wide range of colors using only relatively small quantities of direct dyeing dyestuffs. I have now found that very satisfactory deep dark shades may be produced on materials made of or containing cellulose esters or ethers by incorporating in the materials black dyestuffs. These dyestuffs give to the materials a desirable neutral shade free from red, brown or blue fluorescence or cast. When such neutral grey colored materials are dyed with direct dyeing dyestuffs, deep dark shades which are fast to rubbing are produced. In accordance with my invention, therefore, I produce textile materials having a neutral grey shade by incorporating in said textile materials a small amount of a mixture of black dyestuffs, preferably a mixture of Aniline Black and Alizarin Cyanine Black (Colour Index No. 1065).

Dark shades are produced on the textile materials colored neutral grey in accordance with this invention by dyeing the same with dyestuffs having an affinity for the textile materials. In accordance with the process of this invention, a reduced amount of the direct dyeing dyestuff is necessary to produce desirable deep dark shades on the textile materials. Furthermore, the incorporation of the dyestuffs in the material is particularly easy as the operation may readily be effected by way of the spinning solution from which the materials are produced. This method is of particular value in the production of dark shades upon artificial filaments or yarns of cellulose esters or ethers for, as indicated above, there is for these materials a marked lack of direct dyeing dyestuffs inherently capable of yielding deep shades thereon.

The grey neutral shades produced in accordance with this invention are of particular value in that by applying relatively small quantities of dyestuffs thereto an extremely wide range of deeply colored materials may be produced from

a single material having the black dyestuffs incorporated therein. Thus, in order to produce black shades small amounts only of blue, red and yellow need be applied to the neutral grey material. Moreover, by an application to the same neutral grey material of green or a mixture of blue and yellow dyestuffs there may be produced a series of olive green, khakis, drabs and the like. Where yellows, oranges and reds are applied to the neutral green materials shades varying from yellow brown to chocolate may be obtained, while purple, violet and the like produce wine shades such as, for example, Bordeaux, maroon, etc.

It will be appreciated from the foregoing that for commercial requirements it is not essential, in order to obtain a satisfactory range of deep shades, to manufacture more than a very limited number of neutral grey materials. In fact, two or three materials having different amounts of Alizarin Black dyestuffs therein will be found to be sufficient to cover practically all commercial requirements as regards dark shades.

As previously indicated, my invention is of particular importance in connection with the production of deeply colored cellulose ester or ether material, more particularly on account of the lack of inherently dark dyestuffs for these materials. As examples of such cellulose esters or ethers, especial mention may be made of cellulose acetate and of other organic acid esters of cellulose, for example, cellulose propionate and cellulose butyrate, also ethers of cellulose, e. g., ethyl cellulose and benzyl cellulose. My invention is not, however, limited to the treatment or production of cellulose ester or ether textile materials in the form of filaments or yarns, as it may be applied to cellulose esters or ethers in other forms such as, for example, ribbons, straws or films or like products having a large surface in relation to their mass. The process of my invention may also be applied to textile materials generally, either natural or artificial, and especially to such artificial materials as may be prepared by extrusion of appropriate solutions, for example, regenerated cellulose prepared from viscose, and synthetic linear polyamide condensation products such as the polyamides derived from amino-acids or from the condensation products of diamines with carboxylic acids, e. g. polyhexamethylene adipamide.

As previously indicated, I prefer to use a mixture of Aniline Black and Alizarin Cyanine Black. While these substances may be incorporated in the materials at any stage of production of the latter, I prefer to incorporate the same in the spinning solution from which the filaments of cellulose esters or ethers are spun. The dyestuff mixture or dispersion containing the black dyestuffs which is to be added to the spinning solution is prepared by grinding, rubbing or kneading the dyestuffs in the presence of a derivative of cellulose and a solvent therefor. In this manner the dyestuffs are ground to relatively fine particle size. For example, Alizarin Black dyestuffs, preferably in the form of powders, may be ground in the presence of cellulose acetate dissolved in acetone. The mixture or dispersion so formed has a dyestuff concentration of from 1 to 50%, based on the weight of the cellulose acetate present, the amount of dyestuff depending in part on the viscosity of the cellulose acetate employed. The grinding of the dyestuffs in the presence of the cellulose derivative and solvent produces a dyestuff particle size of such fineness that filtra-

tion other than that supplied by the candle and jet of the spinning apparatus may be eliminated.

In forming the neutral grey colored filaments or yarn there is employed in the spinning solution from 0.3 to 0.9%, and preferably 0.7% based on the weight of the cellulose acetate present, of black dyestuffs. However, lesser or larger amounts may be employed where desired.

In order further to illustrate my invention, but without being limited thereto the following specific examples are given.

#### Example I

20 parts by weight of a mixture of Aniline 15 Black and Alizarin Cyanine Black in powder form is added to a solution containing 40 parts by weight of cellulose acetate dissolved in 360 parts by weight of acetone and the resulting mixture is milled for twenty-four (24) hours in a ball mill. 20 A cellulose acetate spinning solution containing 25% of cellulose acetate dissolved in acetone is then prepared. To this spinning solution is added sufficient of the above dyestuff dispersion to give a dyestuff concentration therein of 0.7% based on the weight of the cellulose acetate. The spinning 25 solution containing the dyestuff without extraneous filtration is spun into filaments by a dry spinning process, producing yarns of a neutral grey color. The neutral grey colored yarns are free from a red, brown, or blue cast and are found to 30 be of substantially the same physical characteristics as those obtained by spinning a solution which is free from the dyestuffs.

#### Example II

The neutral grey yarn obtained by the process of Example I is dyed from a 30 to 1 soap bath containing dispersed therein coloring matters having direct affinity for the cellulose acetate. 40 The yarn is entered into the bath at a relatively low temperature which is gradually increased to 70 to 80° C. and the dyeing continued until the desired shade is achieved. The yarn is then withdrawn from the dye bath, washed, dried and finished in the usual manner. Any of the direct 45 dyeing dyestuffs having affinity for the cellulose acetate may be employed.

It is to be understood that the foregoing detailed description is given merely by way of illustration and that many variations may be made therein without departing from the spirit of my invention.

Having described my invention, what I desire to secure by Letters Patent is:

55 1. A solution for use in the manufacture of neutral grey colored filaments by extruding the same into a setting medium, comprising a cellulose derivative selected from the group consisting of cellulose esters and ethers dissolved in a solvent therefor and containing a dispersion of a mixture of Aniline Black and Alizarin Cyanine Black.

60 2. A solution for use in the manufacture of neutral grey colored filaments by extruding the same into a setting medium, comprising a cellulose acetate dissolved in a solvent therefor and containing a dispersion of a mixture of Aniline Black and Alizarin Cyanine Black.

65 3. A solution for use in the manufacture of neutral grey colored filaments by extruding the same into a setting medium, comprising a cellulose derivative selected from the group consisting of cellulose esters and ethers dissolved in a solvent therefor and containing a dispersion of a mixture of Aniline Black and Alizarin Cyanine

Black in an amount sufficient to give a concentration of between 0.3 and 0.9%, based on the weight of the cellulose derivative present in the solution.

4. A solution for use in the manufacture of neutral grey colored filaments by extruding the same into a setting medium, comprising a cellulose acetate dissolved in a solvent therefor and containing a dispersion of a mixture of Aniline Black and Alizarin Cyanine Black in an amount sufficient to give a concentration of between 0.3 and 0.9%, based on the weight of the cellulose acetate present in the solution. 10

5. A solution for use in the manufacture of neutral grey colored filaments by extruding the same into a setting medium, comprising a cellulose derivative selected from the group consisting of cellulose esters and ethers dissolved in a solvent therefor and containing a dispersion of a mixture of Aniline Black and Alizarin Cyanine 15 20

Black in an amount sufficient to give a 0.7% concentration.

6. A solution for use in the manufacture of neutral grey colored filaments by extruding the same into a setting medium, comprising a cellulose acetate dissolved in a solvent therefor and containing a dispersion of a mixture of Aniline Black and Alizarin Cyanine Black in an amount sufficient to give a 0.7% concentration.

7. Neutral grey colored textile materials comprising materials having a basis of a cellulose derivative selected from the group consisting of cellulose esters and ethers and having incorporated therein a mixture of Aniline Black and Alizarin Cyanine Black.

8. Neutral grey colored textile materials comprising materials having a basis of cellulose acetate and having incorporated therein a mixture of Aniline Black and Alizarin Cyanine Black.

GEORGE SCHNEIDER.